# EUROPEAN PATENT SPECIFICATION

(11) **EP 2 924 131 B1**
(45) Date of publication and mention of the grant of the patent: **21.08.2019**
(21) Application number: 14162191.2
(22) Date of filing: 28.03.2014
(51) Int. Cl.: C21D 6/00, C21D 8/02, C22C 38/00, C22C 38/02, C22C 38/06, C22C 38/42, C22C 38/44, C22C 38/50, C22C 38/54, C22C 38/58

(54) **AUSTENITIC HIGH-MANGANESE STAINLESS STEEL**
HOCHMANGANHALTIGER AUSTENITISCHER EDELSTAHL
ACIER INOXYDABLE AUSTÉNITIQUE À HAUTE TENEUR EN MANGANÈSE

(43) Date of publication of application: 30.09.2015
(73) Proprietor: Outokumpu Oyj, 00180 Helsinki (FI)
(72) Inventor: Breuer, Arno, 50825 Köln (DE); Brückner, Gabriele, 41372 Niederkrüchten (DE); Mosecker, Linda, 52062 Aachen (DE); Bleck, Wolfgang, 52072 Aachen (DE)

(56) References cited:
- EP-A1- 1 069 202
- EP-A1- 2 465 954
- DE-A1-102010 026 808
- DE-C- 728 159
- FR-A5- 2 071 667

## Description

The invention relates to an austenitic high-manganese stainless steel having high strength and high ductility, wherein the stainless steel utilizes the TWIP (TWinning Induced Plasticity) mechanism during the deformation process.

The austenitic stainless steels, such as the most versatile and widely used 304 austenitic stainless steel, have a significantly lower strength combined with relatively high residual elongation after cold deformation, such as cold rolling. The ferritic austenitic duplex stainless steels, such as the 2304 ferritic austenitic duplex stainless steel, offer a high strength, but loose ductility with even a low cold deformation degree.

The austenitic manganese stainless steels with high carbon content are vulnerable to intergranular corrosion after welding in the weld and heat-affected zone due to chromium depletion in this area. Further, the typical manganese stainless steels are in general vulnerable to form martensitic phase after cold deformation, which could lead to delayed cracking.

The FR patent 2071667 relates to a nickel-free austenitic stainless steel which contains weight % 0.02 to 0.3 % carbon, 0.1 to 0.3 % silicon, 12.0 to 16.0 % chromium, 8.0 to 17.0 % manganese, 0.05 to 0.3 % nitrogen, 0.1 to 3.0 % copper, 0.1 to 3.0 % molybdenum, the balance being iron and evitable impurities. The object of the FR patent application 2071667 is to have improved softening and better forming properties. However, based on the chemical composition of the FR patent application 2071667 the manganese (Mn) content should not contain more than 17 weight %, because a higher content produces less austenite phase.

The EP patent application 1069202 describes a method for manufacturing an austenitic, paramagnetic stainless steel and the steel consists, by weight %, of up to about 0.1 % carbon, about 0.21 to about 0.6 % silicon, about 17 to about 24 % chromium, up to about 2.5 % nickel, greater than about 20 % to less than about 30 % manganese, greater than about 0.6 % to less than about 1.4 % % nitrogen, up to about 0.3 % copper, up to about 1.9 % molybdenum, up to about 0.002 % boron, up to about 0.8 % carbide-forming elements, such as titanium, zirconium, vanadium and niobium, the balance being iron and evitable impurities. Manganese is provided to increase the nitrogen solubility and to stabilize the austenitic and/or ferrite-free microstructure. According to the method, the material is hot-formed at a temperature of at least 850 °C to a degree of deformation of at least about 3,5 times and actively cooled. In the second step it is cold-formed in a deformation of 5 - 20 % below the deposit temperature of nitrides at elevated temperature below 600 °C, but greater than 350 °C. In order to avoid martensite formation the deformation is in every process step thus carried out at an elevated temperature which increases the manufacturing costs of the produced material. A twinning in the microstructure of a metal material is in general defined as two separate crystals that share some of the same crystal lattice. The TWIP (TWinning Induced Plasticity) stainless steels have austenitic microstructure with face-centered cubic lattice (FCC) along with a relatively low stacking fault energy (SFE) promoting the activation of twinning deformation mechanism, i.e. mechanically induced twinning in the crystal lattice. The term TWIP indicates that twinning often goes along with accomodation plasticity via lattice dislocations.

The object of the present invention is to eliminate some drawbacks of the prior art and to achieve an improved austenitic high-manganese stainless steel which utilizes the TWIP (TWinning Induced Plasticity) mechanism in the cold deformation in order to have a high work-hardening rate and good corrosion resistance with low vulnerability for intergranular corrosion after welding and for delayed cracking and stress corrosion cracking. The essential features of the austenitic stainless steel are enlisted in the appended claims.

According to the invention the austenitic high-manganese stainless steel consists of in weight % 0,03 - 0,1 % carbon, 0,08 - 1,0 % silicon, 14 - 26 % manganese. 10,5 - 18 % chromium, less than 0,8 % nickel, 0,05 - 0,6 % copper, 0,1 - 0,8 % nitrogen and 0,0008 - 0,005 % boron, the rest being iron and inevitable impurities occurred in stainless steels. The austenitic stainless steel of the invention further contains optionally 0,001 - 0,02 % titanium and optionally less than 0,04 % aluminium. The austenitic stainless steel of the invention has a superior ductility and high strength after plastic deformation utilizing in the cold deformation the TWIP (TWinning Induced Plasticity) mechanism. The austenitic stainless steel of the invention combines thus a high strength in the initial annealed state and a high work hardening rate with a high elongation after the cold deformation, such as cold rolling, in connection with a low nickel content.

The ranges for the yield strength R_{p0,2} and the tensile strength Rₘ as well as the elongation to fracture A₈₀ at the annealed state the austenitic high-manganese stainless steel in accordance with the invention are 470 - 600 MPa for R_{p0,2}, 800 - 930 MPa for Rₘ and 40 - 60 % for A₈₀ after annealed at the temperature range of 1000 - 1150 °C. When the austenitic stainless steel in accordance with the invention was further cold deformed, such as cold rolled, the effect of TWIP (TWinning Induced Plasticity) mechanism can be shown by means of the respective ranges for the yield strength R_{p0,2} and the tensile strength Rₘ as well as the elongation to fracture A₈₀ enlisted in the following table 1 after the cold rolling with the reduction degrees of 10 % and 20 %:

**Table 1**

| Deformation degree | R_{p0,2} (MPa) | Rₘ (MPa) | A₈₀ (%) |
|---|---|---|---|
| 10 % | 800-900 | 900-1030 | 25 - 35 |
| 20 % | 1000-1100 | 1100-1250 | 10 - 20 |

The austenitic high-manganese stainless steel of the invention has a high work-hardening rate of at least 20 % with the deformation degree 10 % and at least 40 % with the deformation degree 20 % for the yield strength R_{p0,2}. Further, the elongation to fracture A₈₀ is 25 - 35 % with the deformation degree 10 % and 10 - 20 % with the deformation degree 20 % showing the good ductility.

The effects of the main elements in the chemical composition of the austenitic high-manganese stainless steel according to the invention are described, the ranges being in weight %, if not otherwise mentioned.

Carbon (C) is a valuable austenite forming and stabilizing element, which enables reduced use of expensive elements nickel and copper. The upper limit for carbon alloying (less than 0,1 %) is set by the risk of carbide precipitation, which deteriorates the corrosion resistance of the stainless steel. The carbon content is low enough to maintain good corrosion resistance. The reduction of the carbon content to low levels by the decarburization process is non-economical, and therefore, the carbon content shall not be less than 0,03 %.

Silicon (Si) is added to stainless steels for deoxidizing purposes during melting and should not be below 0,08 %. Because silicon is a ferrite forming element, its content must be limited below 1 %.

Manganese (Mn) is a key element of the austenitic stainless steel of the invention, ensuring the stable austenitic crystal structure and enabling the twinning mechanism and, further, the reduction of the use of more expensive nickel. Manganese also increases the solubility of nitrogen to the stainless steel. Plastic deformation accompanied with twinning deformation easily occurs in the case of an amount of manganese of 14 % or more without deformed structure, i.e. the strain-induced martensite. A high manganese content makes the decarburization process of the steel more difficult, impairs the surface quality and reduces the corrosion resistance of the steel. Therefore the manganese content shall be less than 26 %.

Chromium (Cr) is responsible of ensuring corrosion resistance of a stainless steel. Therefore, the chromium content in this stainless steel shall be at the minimum 10,5 %. Chromium is important in terms of avoiding the delayed cracking phenomenon. By increasing the content from this level the corrosion resistance of the steel can be improved. However, because chromium is a ferrite forming element, the increasing of the chromium content increases the need for expensive austenite formers, such as nickel and manganese or necessitates impractically high carbon and nitrogen contents. Therefore, the chromium content shall be lower than 18 %. Chromium also increases the solubility of nitrogen.

Nickel (Ni) is a strong austenite former and stabilizer, but nickel is an expensive element. However, very low nickel contents would necessitate impractically high alloying with the other austenite forming and stabilizing elements. Therefore, the nickel content shall be preferably lower than 0,8 % but preferably less than 0,5 %.

Copper (Cu) is present as a residual of 0,1 - 0,6 %. Copper is a weak stabilizer of the austenite phase but, however, has a strong effect on the resistance to martensite formation. Copper also has a positive effect on ductility and forming properties.

Nitrogen (N) is a strong austenite former and stabilizer. Therefore, nitrogen alloying improves the cost efficiency of the steel by enabling lower use of nickel and copper. In order to ensure reasonably low use of the above-mentioned alloying elements, nitrogen content shall be at least 0,1 %. High nitrogen contents increase the strength of the steel and thus make forming operations more difficult. Furthermore, risk of nitride precipitation increases with increasing nitrogen content. For these reasons, the nitrogen content shall not exceed 0,8 %, preferably the nitrogen content shall be lower than 0,6 %. Nitrogen increases the stacking fault energy (SFE), which is used for the prediction of the TWIP-effect, and thus enables for and facilitates the TWIP-effect.

The austenitic stainless steel according to the invention does not form during cold rolling any deformation martensite at the room temperature or above. Therefore, the stainless steel of the invention has a high ductility. The austenitic stainless steel according to the invention is also free of stress corrosion cracking and delayed cracking, just even after aging process in air and also in 5 % sodium chloride (NaCl) environment.

### Example

The austenitic stainless steel in accordance with invention was melted in the production scale and then cast into a slab form with the chemical composition in weight %, where the Mo-content of 0.02% is an accidental impurity.

**Table 2**

| C | Si | Mn | Cr | Mo | Ni | Ti | Cu | Al | N | B |
|---|---|---|---|---|---|---|---|---|---|---|
| 0.08 | 0.5 | 20 | 13 | 0.02 | 0.2 | 0.003 | 0.5 | 0.01 | 0.43 | 0.0023 |

The slabs were further hot rolled into the thickness of 4,0 mm and then annealed at the temperature 1080 °C. The austenitic stainless steel of the invention was further cold rolled with the rolling degree of 50 % to the thickness of 2,0 mm and annealed at the temperature 1080 °C. The annealed strip product was then tested by determining the yield strength R_{p0,2} and the tensile strength Rₘ as well as the elongation to fracture A₈₀.

In order to utilize the TWIP effect in the austenitic stainless steel of the invention the stainless steel strip was cold deformed with the reduction degree of 10 % and then determined the yield strength R_{p0,2} and the tensile strength Rₘ as well as the elongation to fracture A₈₀. The respective actions were also made for the cold deformed strip having the reduction degree of 20 %. The results for those test results are described in the following table:

**Table 3**

| Reduction degree | R_{p0,2} (MPa) | Rₘ (MPa) | A₈₀ (%) |
|---|---|---|---|
| 0 % | 500 | 830 | 48 |
| 10 % | 800 | 950 | 28 |
| 20 % | 1020 | 1180 | 14 |

The results show that the austenitic stainless steel in accordance with the invention has high work-hardening rate for the yield strength R_{p0,2}. Further, the elongation to fracture A₈₀ is 28 % with the deformation degree 10 % and 14 % with the deformation degree 20 % shows still a good ductility at high strength after cold rolling.

The austenitic stainless steel of the invention can be manufactured as slabs, blooms, billets and flat products such as coils, strips, plates, sheets, and long products such as bars, rods, wires, profiles and shapes, and tubular products such as pipes, tubes and can be applied for instance in automotive construction, tanks and crash relevant parts, construction and rail vehicles.

The high-manganese austenitic stainless steel in accordance with the invention can be cold deformed in the state of as hot strip annealed, as cold strip annealed and as hot and cold strip annealed and cold rolled in order to utilize the TWIP effect for higher yield and tensile strength values with still high ductility.

## Claims

1. Austenitic high-manganese stainless steel having high strength and ductility, **characterized in that** the stainless steel which consists, by weight %, of 0,03 - 0,1 % carbon, 0,08 - 1,0 % silicon, 14 - 26 % manganese. 10,5 - 18 % chromium, less than 0,8 % nickel, 0,05 - 0,6 % copper, 0,1 - 0,8 % nitrogen and 0,0008 - 0,005 % boron, the rest being iron and inevitable impurities occurring in stainless steels, optionally 0,001 - 0,02 % titanium and optionally less than 0,04 % aluminium; and which in the state of being annealed in the temperature range of 1000 - 1150 °C, the ranges for the yield strength R_{p0,2} and the tensile strength Rₘ as well as the elongation to fracture A₈₀ are 470 - 600 MPa for R_{p0,2}, 800 - 930 MPa for Rₘ and 40 - 60 % for A₈₀, and the steel being cold deformable utilizing the TWIP or TWinning Induced Plasticity mechanism so that the work-hardening rate based on a cold deformation degree of 10% for the yield strength R_{p0,2} is at least 20 %.

2. Austenitic high-manganese stainless steel according to the claim 1, **characterized in that** the work-hardening rate based on the cold deformation degree of 20% for the yield strength R_{p0,2} is at least 40 %.

3. Austenitic high-manganese stainless steel according to any of the preceding claims, **characterized in that** elongation to fracture A₈₀ is 25 - 35 % with the cold deformation degree 10 %.

4. Austenitic high-manganese stainless steel according to any of the preceding claims, **characterized in that** elongation to fracture A₈₀ is 10-20 % with the cold deformation degree 20 %.

5. Austenitic high-manganese stainless steel according to any of the preceding claims, **characterized in that** the stainless steel is cold deformable for the TWIP effect in the state of as hot-rolled strip annealed at the temperature range of 1000 - 1150 °C.

6. Austenitic high-manganese stainless steel according to any of the preceding claims 1 - 4, **characterized in that** the stainless steel is cold deformable for the TWIP effect in the state of as cold-rolled strip annealed at the temperature range of 1000 - 1150 °C.

7. Austenitic high-manganese stainless steel according to any of the preceding claims 1 - 4, **characterized in that** the stainless steel is cold deformable for the TWIP effect in the state of as hot and cold strip annealed at the temperature range of 1000 - 1150 °C and cold rolled.

8. Austenitic high-manganese stainless steel according to any of the preceding claims, **characterized in that** the austenitic stainless steel is manufactured as slabs, blooms, billets, flat products such as coils, strips, plates, sheets, long products such as bars, rods, wires, profiles and shapes, tubular products such as pipes, tubes.

9. Austenitic high-manganese stainless steel according to any of the preceding claims, **characterized in that** the austenitic stainless steel is applied for instance in automotive construction, tanks and crash relevant parts, construction and rail vehicles.

## Patentansprüche

1. Austenitischer hochmanganhaltiger rostfreier Stahl mit hoher Festigkeit und Duktilität, **dadurch gekennzeichnet, dass** der rostfreie Stahl, in Gewichts-%, aus 0,03 bis 0,1 % Kohlenstoff, 0,08 bis 1,0 % Silicium, 14 bis 26 % Mangan, 10,5 bis 18 % Chrom, unter 0,8 % Nickel, 0,05 bis 0,6 % Kupfer, 0,1 bis 0,8 % Stickstoff und 0,0008 bis 0,005 % Bor, wobei der Rest Eisen und unvermeidbare Verunreinigungen sind, die in rostfreien Stählen vorkommen, gegebenenfalls 0,001 bis 0,02 % Titan und gegebenenfalls unter 0,04 % Aluminium besteht; und im Zustand des Glühens im Temperaturbereich von 1000 bis 1150 °C die Bereiche für die Streckgrenze R_{p0,2} und die Zugfestigkeit Rₘ sowie die Bruchdehnung A₈₀ 470 bis 600 MPa für R_{p0,2}, 800 bis 930 MPa für Rₘ und 40 bis 60 % für A₈₀ lauten, und der Stahl unter Verwendung des TWIP-Mechanismus oder Mechanismus der durch Zwillingsbildung induzierten Plastizität kaltverformbar ist, sodass die Kaltverfestigungsgeschwindigkeit auf Grundlage eines Kaltverformungsgrads von 10 % für die Streckgrenze R_{p0,2} mindestens 20 % beträgt.

2. Austenitischer hochmanganhaltiger rostfreier Stahl nach Anspruch 1, **dadurch gekennzeichnet, dass** die Kaltverfestigungsgeschwindigkeit auf Grundlage des Kaltverformungsgrads von 20 % für die Streckgrenze R_{p0,2} mindestens 40 % beträgt.

3. Austenitischer hochmanganhaltiger rostfreier Stahl nach einem der vorhergehenden Ansprüche, **dadurch gekennzeichnet, dass** die Bruchdehnung A₈₀ 25 bis 35 % beim Kaltverformungsgrad von 10 % beträgt.

4. Austenitischer hochmanganhaltiger rostfreier Stahl nach einem der vorhergehenden Ansprüche, **dadurch gekennzeichnet, dass** die Bruchdehnung A₈₀ 10 bis 20 % beim Kaltverformungsgrad von 20 % beträgt.

5. Austenitischer hochmanganhaltiger rostfreier Stahl nach einem der vorhergehenden Ansprüche, **dadurch gekennzeichnet, dass** der rostfreie Stahl im Zustand als warmgewalztes Band, das im Temperaturbereich von 1000 bis 1150 °C geglüht wurde, für den TWIP-Effekt kaltverformbar ist.

6. Austenitischer hochmanganhaltiger rostfreier Stahl nach einem der vorhergehenden Ansprüche 1 bis 4, **dadurch gekennzeichnet, dass** der rostfreie Stahl im Zustand als kaltgewalztes Band, das im Temperaturbereich von 1000 bis 1150 °C geglüht wurde, für den TWIP-Effekt kaltverformbar ist.

7. Austenitischer hochmanganhaltiger rostfreier Stahl nach einem der vorhergehenden Ansprüche 1 bis 4, **dadurch gekennzeichnet, dass** der rostfreie Stahl im Zustand als Warm- und Kaltband, das im Temperaturbereich von 1000 bis 1150 °C geglüht wurde, und im Zustand des Kaltwalzens für den TWIP-Effekt kaltverformbar ist.

8. Austenitischer hochmanganhaltiger rostfreier Stahl nach einem der vorhergehenden Ansprüche, **dadurch gekennzeichnet, dass** der austenitische rostfreie Stahl als Brammen, Blöcke, Knüppel, Flachprodukte wie Bunde, Bänder, Platten, Bleche, Langprodukte wie Stäbe, Stangen, Drähte, Profile und Träger, Rohrprodukte wie Rohre, Röhren hergestellt ist.

9. Austenitischer hochmanganhaltiger rostfreier Stahl nach einem der vorhergehenden Ansprüche, **dadurch gekennzeichnet, dass** der austenitische rostfreie Stahl beispielsweise im Fahrzeugbau, bei Behältern und crashrelevanten Teilen, im Baugewerbe und bei Schienenfahrzeugen angewendet wird.

## Revendications

1. Acier inoxydable austénitique à teneur en manganèse élevée ayant une résistance et ductilité élevées, **caractérisé en ce que** l'acier inoxydable est constitué, en pourcentage massique, entre 0,03 et 0,1 % de carbone, entre 0,08 et 1,0 % de silicium, entre 14 et 26 % de manganèse, entre 10,5 et 18 % de chrome, moins de 0,8 % de nickel, entre 0,05 et 0,6 % de cuivre, entre 0,1 et 0,8 % d'azote et entre 0,0008 et 0,005 % de bore, le reste étant du fer et des impuretés inévitables survenant dans les aciers inoxydables, éventuellement entre 0,001 et 0,02 % de titane et éventuellement moins de 0,04 % d'aluminium; et qui se trouve dans l'état de recuit dans la plage de températures comprises entre 1000 et 1150°C, les plages pour la limite d'élasticité R_{p0,2} et la tensions de traction Rₘ ainsi que l'allongement total à la rupture A₈₀ sont comprises entre 470 et 600 MPa pour R_{p0,2}, entre 800 et 930 MPa pour Rₘ et entre 40 et 60 % pour A₈₀, et l'acier pouvant être déformé à froid en utilisant le TWIP ou le mécanisme de plasticité induite par le jumelage de sorte que le taux d'écrouissage en fonction d'un degré de déformation à froid de 10 % pour la limite d'élasticité R_{p0,2} est d'au moins 20 %.

2. Acier inoxydable austénitique à teneur en manganèse élevée selon la revendication 1, **caractérisé en ce que** le taux d'écrouissage en fonction du degré de déformation à froid de 20 % pour la limite d'élasticité R_{p0,2} est d'au moins 40 %.

3. Acier inoxydable austénitique à teneur en manganèse élevée selon l'une quelconque des revendications précédentes, **caractérisé en ce que** l'allongement total à la rupture A₈₀ est compris entre 25 est 35 ayant un degré de déformation à froid de 10 %.

4. Acier inoxydable austénitique à teneur en manganèse élevée selon l'une quelconque des revendications précédentes, **caractérisé en ce que** l'allongement total à la rupture A₈₀ est compris entre 10 et 20 ayant un degré de déformation à froid de 20 %.

5. Acier inoxydable austénitique à teneur en manganèse élevée selon l'une quelconque des revendications précédentes, **caractérisé en ce que** l'acier inoxydable peut être déformé à froid pour l'effet TWIP dans l'état de recuit de bande laminée à chaud à la plage de températures comprises entre 1000 et 1150 °C.

6. Acier inoxydable austénitique à teneur en manganèse élevée selon l'une quelconque des revendications 1 à 4 précédentes, **caractérisé en ce que** l'acier inoxydable peut être déformé à froid pour l'effet TWIP dans l'état de recuit de bande laminée à froid à la plage de températures comprises entre 1000 et 1150 °C.

7. Acier inoxydable austénitique à teneur en manganèse élevée selon l'une quelconque des revendications 1 à 4 précédentes, **caractérisé en ce que** l'acier inoxydable peut être déformé à froid pour l'effet TWIP dans l'état de recuit laminé à chaud et à froid à la plage de températures comprises entre 1000 et 1150 °C et laminé à froid.

8. Acier inoxydable austénitique à teneur en manganèse élevée selon l'une quelconque des revendications précédentes, **caractérisé en ce que** l'acier inoxydable austénitique est fabriquée sous forme de dalles, de blooms, de billets, de produits plats tels que des bobines, des bandes, des plaques, des feuilles, de produits longs tels que des barres, des tiges, des câbles, des profilés et des formes, des produits tubulaires tels que des tuyaux et des tubes.

9. Acier inoxydable austénitique à teneur en manganèse élevée selon l'une quelconque des revendications précédentes, **caractérisé en ce que** l'acier inoxydable austénitique s'applique par exemple dans la construction automobile, dans les parties pertinentes de tanks et d'accidents, et dans les véhicules de construction et sur rail.
